

## UNITED STATES PATENT OFFICE

WILLIAM COTTON, OF HOCHST-ON-THE-MAIN, GERMANY, ASSIGNOR TO GENERAL ANILINE WORKS, INC., OF NEW YORK, N. Y., A CORPORATION OF DELAWARE

## PROCESS FOR PRODUCING FAST COLORED RESISTS UNDER ANILINE BLACK

No Drawing. Application filed January 28, 1926, Serial No. 84,510, and in Germany February 5, 1925.

Many attempts have already been made to produce fast colored resists under aniline black by means of vat dyestuffs. However, such resists could not be widely adopted in practice because they are apt to form halos.

Now I have found that the above-mentioned draw-back can be easily avoided by treating the goods with a padding bath such as is generally used for dyeing with aniline black, printing on them enol esters of vat dyestuffs to which compounds giving an acid reaction on steaming without tendering the fiber are added, and then finishing the goods in the manner practiced in the production of aniline black. It could not be foreseen that under the above stated conditions the enol esters can be oxidized more easily than aniline and that consequently they are suitable for the production of colored resists under aniline black.

The following example illustrates my invention:

The printing-color is prepared as follows:

80 gr. of enol ester of 5-7-5'-7'-tetrabromindigo, (Schultz, Farbstofftabellen, 6th ed., vol. 1, page 300, No. 881).

370 gr. of water

500 gr. of neutral wheat-starch tragacanth thickening

50 gr. of neutral ammonium oxalate

1 kilo.

This color is printed on the material padded with aniline, whereupon the material is steamed for 3 minutes, passed through a weak bath of potassium bichromate, washed and soaped.

I claim:

1. Process for producing fast colored resists under aniline black, which consists in printing on the goods, previously treated with a padding-bath as it is generally used in the dyeing with aniline black, enol esters of vat dyestuffs to which are added compounds which give an acid reaction on steaming with-

out tendering the fiber and then finishing the goods in the manner practiced in the production of aniline black.

2. Process of producing fast colored resists under aniline black, which comprises printing on goods, previously treated with a padding-bath as it is generally used in the dyeing with aniline black, an enol ester of 5-7-5'-7'-tetrabromindigo to which is added a compound which gives an acid reaction on steaming without tendering the fiber, and then finishing the goods in the manner practiced in the production of aniline black.

In testimony whereof, I affix my signature.

WILLIAM COTTON.

60

50

55

50

55

55

65

70

70

75

80

85

85

90